

April 29, 1924.

1,491,881

J. E. PERRY

METHOD, MOLD, AND INGOT

Filed Oct. 21, 1920



Fig. 1.



Fig. 2.



Fig. 3.



Fig. 4.



Fig. 5.



Fig. 6.



Fig. 7. John E. Perry  
Inventor

By 6 George Ramsey  
Attorney

## UNITED STATES PATENT OFFICE.

JOHN E. PERRY, OF SHARON, PENNSYLVANIA, ASSIGNOR TO VALLEY MOULD AND IRON CORPORATION, OF SHARPSVILLE, PENNSYLVANIA, A CORPORATION OF NEW YORK.

## METHOD, MOLD, AND INGOT.

Application filed October 21, 1920. Serial No. 418,398.

*To all whom it may concern:*

Be it known that I, JOHN E. PERRY, a citizen of the United States, and a resident of the city of Sharon, in the county of Mercer, 5 State of Pennsylvania, have invented new and useful Improvements in Methods, Molds, and Ingots, of which the following is a specification.

The present invention relates broadly to 10 metallurgy and more specially to a method, a mold and a steel ingot.

The principal object of the present invention is the method of producing a steel ingot, the mold for carrying out the method, 15 and the ingot resulting from the method, wherein a smooth ingot is formed with a substantially uniform chilled shell enclosing any gas bubbles that may develop during cooling and with the gas bubbles deep seated 20 in the ingot.

Another object of the present invention is an ingot of steel or the like comprising a chilled shell of steel enclosing any gas bubbles that may form during cooling with the 25 thickness of the shell sufficient to prevent the gas bubbles from breaking out during rolling.

A further object of the present invention is the production of a steel ingot or the like 30 having a chilled shell enclosing any gas bubbles that may form during cooling and with the general direction of the length of such gas bubbles being at substantially right angles to the shell wall adjacent said bubbles.

35 A further object of the present invention is a steel ingot as an article of manufacture comprising an ingot having all sides thereof uniformly chilled and with the chilled zones comprising longitudinal closed areas, the 40 maximum area comprising the surface of the ingot and the minimum area comprising a closed zone located adjacent the longitudinal axis of the ingot.

Another object of the present invention is 45 an ingot as an article of manufacture comprising a horizontal ingot having all surfaces thereof chilled to a substantially uniform depth and with the elements of the ingot having the lowest point of fusion located in the central longitudinal portion of 50 the ingot.

A still further object of this invention is the production as an article of manufacture

of an ingot of steel or the like comprising a longitudinal ingot having all surfaces thereof chilled, having the metal therein substantially symmetric with reference to the ends of the ingot and with the metal containing ingredients of the highest point of fusion being adjacent the surface of the ingot and 60 with the metal containing the ingredients of lower points of fusion being located in the interior of the ingot.

A still further object of the present invention is the method of casting steel ingots in 65 such manner that the highest portion of the mold comprises a part other than a flat side thereof.

Another object of the present invention is the method of casting steel ingots in such 70 manner that a corner of the ingot comprises the highest part of the mold during the part of the molding operation when gases are being expelled from the steel.

Another object of the present invention is 75 a horizontal ingot mold with one diagonal plane of the mold being substantially a vertical plane.

Another object of the present invention is the method of casting steel ingots by causing 80 the surface area of the molten steel to widen from the bottom of the mold upwardly to a predetermined zone and then to gradually narrow as the metal fills the mold, until the final portion of the mold is substantially the apex of an angular surface.

A still further object of the present invention is the method of casting steel ingots which comprises casting the ingot with the major axis thereof substantially horizontal 90 and with the pool of molten steel forming the ingot having a surface which gradually widens as the mold is filled from the bottom to a predetermined point, and then the surface gradually narrows from said predetermined point to the upper extremity of the mold, while permitting gases to escape from the portion of the mold which forms the highest part of the ingot.

Another object of the present invention 100 is the method of casting steel ingots which comprises casting the ingot horizontally, causing the upper surface of the molten steel as it fills the mold to gradually narrow until the surface becomes substantially a line 105 formed by the intersection of angularly dis-

posed sides, and chilling the sides of the ingot during the casting operation.

Another object of the present invention is the method of casting a steel ingot with the major axis thereof substantially horizontal and with a diagonal plane thereof substantially vertical, and permitting gases to escape from the mold during the casting operation at a point or points located in said 10 vertical diagonal plane.

A further and important object of the present invention is a horizontal mold for carrying out the process specified, which mold comprises a multi-part structure having the major axis of the matrix portion substantially horizontal and with a diagonal of the matrix portion substantially vertical, whereby the highest part of the matrix portion comprises an angle formed by the intersection 20 of side walls of the mold, and with means being provided adjacent the said intersection to permit escape of gases from the mold.

Other and further objects of the present 25 invention will in part be obvious and will in part be pointed out hereinafter in the specification by reference to the accompanying drawings forming a part of this application and wherein like parts are represented by like characters throughout the several 30 figures thereof.

Realizing that the present invention may be embodied and carried out in constructions and by manipulations other than those herein described I desire that the disclosure here- 35 with shall be considered as illustrative and not in the limiting sense.

Figure 1 is a view diagrammatically illustrating one form of mold embodying the 40 present invention;

Figure 2 is a section on line 2—2 of Figure 1;

Figure 3 is a plan view of Figure 1, illustrating the gas outlets and showing the foun- 45 tain removed;

Figure 4 is a cross-section through a mold having a vertical separation plane;

Figure 5 is a cross-section through a mold having one side removable;

Figure 6 is a longitudinal section through an ingot in accordance with the present invention taken on line 6—6 of Figure 7;

Figure 7 is a cross-section through an ingot in accordance with the present invention taken on line 7—7 of Figure 6.

Heretofore in the steel industry ingots have been cast in various types of horizontal molds and various provisions have been suggested for maintaining the upper portion 60 of the molten steel hot. Under such conditions it appears that the materials which tend to segregate in the cooling of the steel are driven toward the top and undesirable conditions may arise under certain circum- 65 stances.

It has been suggested in the art that steel ingots be cast in chill molds having light chill covers. It has been found that where ingots are cast in trough like chill molds with light chill covers the top surface of the 70 steel, when coming in contact with the cover, tends to chill and form a skin, then gases being expelled from the steel during cooling become trapped beneath this skin. These gases form bubbles which build up in a 75 downward direction and may form large subcutaneous cavities. This condition is aggravated in large ingots because the chilling effect is very slight as compared to the mass of steel in the ingot and the freed gases are 80 relatively large as compared to the chill skin formed by the chill. These subcutaneous cavities break out in rolling and are very undesirable. Furthermore, in the trough type of ingot mold it was necessary to incline 85 the side walls of the molds slightly so that the top of the ingot would be slightly wider than the bottom to provide clearance so that the ingot might be stripped from the mold. It is desirable, for rolling operations, to have 90 the sides of the ingot substantially parallel and the angles necessary for clearance in the trough mold prevented attaining this desired cross-sectional form. It has been proposed, to provide ingot molds with removable sides. Such molds, however, usually require a number of pieces, and often require luting the 95 joints to prevent leakage of steel during casting.

The present invention comprising the 100 method an ingot, and a mold, overcomes the difficulties of the known art by providing for the production of an ingot wherein the chill is proportioned around the ingot in such manner as to be substantially uniform 105 and preferably is a quick chill so that a relatively deep mass of solidified steel is quickly formed around the ingot and wherein the entire ingot may be rolled into finished product. This invention may be carried out in 110 various ways but in the preferred method it is carried out by utilizing an ingot mold with all sides thereof formed of chill metal having a relatively large heat absorbing capacity. Preferably the mold is provided 115 with means for gas escape at the highest portion of the mold so that when the mold is filled with molten steel the free gases are driven ahead of the liquid surface until the mold is filled, at which time the walls of the 120 mold quickly absorb heat from the molten steel, thereby quickly forming a closed shell of solid and plastic steel which encloses a mass of liquid steel that is in the center of the shell. The mold side walls are so proportioned as to cause the chilling operation to take place with sufficient rapidity to establish conditions within the interior of the 125 ingot which prevent the formation of gas bubbles to any serious extent during the cool- 130

ing of the ingot. It appears that under certain circumstances a solid steel shell will form to the depth of 1½ inches or more and then a zone may form including relatively small gas cavities, and the interior of the ingot from that point appears to be substantially solid metal. These deep seated gas bubbles in no way interfere with the production of perfect steel articles from the ingot because it appears in rolling the gas in these cavities, being under pressure, is absorbed in the hot metal and the walls of the cavities weld together. When molten steel is poured into the mold the ingredients of the steel having the highest point of fusion solidify first and this material is substantially the pure steel, so that the parts which solidify first; namely the exterior enclosing shell, is formed substantially of pure steel. As the solidification continues to take place there is a tendency to drive inward materials which fuse at a lower temperature. As the pressure increases, however, on the interior molten steel, the segregation of these elements appears to decrease so that while the shell of the ingot is the purer steel, the interior of the ingot is good metal of a relatively uniform constituency in which is intermingled the lower melting point elements such as phosphorus, sulphur, manganese, etc. It also appears that such gas bubbles as do appear within the outer steel shell, are elongated bubbles which extend in a general direction at right angles to the adjacent chilled side. When the ingot lengthens out under the rolls these bubble cavities tend to turn and incline in the direction of the length of the fiber of the steel thereby receiving a kneading action which assists in closing the cavities. In one way of carrying out this invention the ingot is cast with the major axis of the ingot substantially horizontal and with the diagonal thereof substantially vertical so that the highest portion of the mold is represented by the apex of an angle formed by surfaces of the mold. This construction permits the escape of expelled gases through one end of the mold and in the form where the mold is parted vertically, the parting joint provides an air space through which the expelled gases may escape up to the final moment of solidification. However this same result is accomplished by inclining the mold toward the gas outlet. The present invention, which contemplates parting the mold on a diagonal thereof, permits the sides of the mold matrix to be made in the form of horizontal planes, which produces an ingot having substantially parallel sides and which is better adapted for rolling than the tapered ingot of the type usually made in vertical molds.

In carrying out the present invention it is not absolutely essential that the sides of the ingots shall be plane surfaces because under some circumstances it is desirable that the sides be curved, but in such cases where the sides are curved it is preferable that the mold be set or formed in such manner that the interior longitudinal surfaces at the top of the mold will form an inverted V-section with the apex of the V at the highest part of the mold and with the apex angle as acute an angle as the section of the required mold will permit. It is also desirable that the two surfaces forming the above mentioned apex angle shall have about an equal angle to the horizontal. This approximate equality need not be observed when more gases seem to become entangled on one surface than on the other due to some lack of cross-sectional symmetry in the matrix portion of the mold. In such a case the angle of the surface which tends to hold the most gases may be increased somewhat with reference to the horizontal. In no case, however, should one surface be favored over the other to such an extent as to bring the latter surface to substantially a horizontal plane.

In closed chill molds for carrying out the present invention the ingot is removed broadside from the mold so consequently the mold requires at least two parts. The longitudinal plane of separation may be arranged as desired but preferably is arranged on a vertical plane so that when the steel is poured an outlet for the gases is maintained at the highest part of the mold. While the separation opening may be of sufficient size to permit the escape of gases it should not be sufficiently large to permit the escape of the steel or the forming of a steel fin of appreciable thickness. Hot steel chills, however, before it will enter into a thin or narrow joint, so that joints that are far from air tight are entirely satisfactory so far as escape of steel is concerned. It will be noted the separation joint is the full length of the ingot and therefore is relatively long while the amount of released gas is comparatively small, so therefore a very complete escape of gases occurs where the plane of separation is arranged vertically.

Referring now to the drawings and more specially to Figures 1, 2 and 3, which illustrate one form of mold for carrying out the present invention, the mold may comprises multi-part constructions but preferably comprises two parts such as a lower part 1 and an upper part 2 with the matrix 4 thereof preferably comprising a form with smooth sides forming a rectangle in cross-section. Preferably the corners are slightly rounded in order to prevent sharp angular corners on the ingot. The matrix portion 4 of the ingot is arranged preferably in such manner that one diagonal thereof is vertical and the other diagonal thereof is horizontal.

The major axis of the matrix portion is preferably inclined slightly to the horizontal with the inclination toward the gas outlet presently to be described.

5 The walls around the matrix portion are thickened at the sides thereof in order to increase the heat absorbing capacity and produce a deep uniform chill in the ingot. Preferably the thinnest portion of the wall 10 is adjacent the corners of the matrix which include the horizontal diagonal. The two portions of the mold may be held together by suitable clamps 5 which are adapted to engage lugs formed on the body portions of 15 the mold. One end of the mold is raised and provided with an opening 6 in which a runner of fire clay or the like is adapted to be set. This runner is provided with a lower inlet opening 7 and an upper inlet 20 opening 8. A suitable fountain 9 is mounted above the runner in such manner as to guide molten steel into the opening in the runner. The body of the runner preferably is slightly smaller than the opening 25 in the mold so that gas outlet passageways 10 and 11 are provided around the runner and connecting gas outlet openings 12 and 14 are provided beneath the fountain. These connecting openings are arranged to 30 discharge over the mold and on each side thereof in order that the flames therefrom may be observed by the workmen. The upper portion of the mold may be provided with a suitable lifting staple 15 and the 35 lower portion with suitable supporting legs 16 and 17 which are so proportioned as to slightly incline the axis of the mold toward the end provided with the gas outlet openings. When molten steel is poured into the 40 runner the initial escape of the steel is from the outlet opening 7 and the flow is substantially parallel to the axis of the matrix portion so that the steel strikes the mold some distance from the runner opening 7 45 and immediately forms a chilled skin on which the continuing steel pours so that the hot steel does not cut away the walls of the cast iron chill mold. As the mold fills the gases comprising the original air in the 50 matrix and the gases being expelled during cooling of the steel, rise into the matrix space above the surface of the steel and in view of the fact that gas passages are provided around the runner, the gas escapes 55 through these passages and comes out beneath the fountain through the conduits provided. These passages while ample for the gas escape are sufficiently narrow to prevent any appreciable amount of steel flowing 60 around the runner. As the ferro-static pressure increases in the mold the steel begins to flow from the opening 8. The general direction of movement of the steel in the mold, however, is upward and the direction of the escape of gases is toward the 65 highest end of the mold, which is the runner end. As the molten steel continues to flow into the mold the surface of the steel begins to widen out as the steel surfaces rises from the bottom of the mold until the 70 portion of the mold matrix represented by the horizontal diagonal is reached and from that point on the surface of the molten steel decreases in area. The incline of the sides of the mold and the upward flow of the 75 molten steel tends to sweep away gases which otherwise would collect under the upper portions of the matrix walls so that as the steel rises and flows upwardly and inwardly along the inclined walls the gases 80 in the molten steel are swept out and escaping through the surface of the molten steel are then driven from the mold cavity out through the gas outlets. The end of the matrix farthest from the gas outlet being 85 lower, is filled first and as the teeming is continued the line of contact of molten steel with the final surfaces of the matrix moves from the farther end toward the gas outlet which is adjacent the runner 8 and therefore is adjacent the hot molten steel last to come into the mold. This provides that 90 gases may escape through the hot molten steel and the outlet up to the moment the mold is entirely filled. Consequently substantially all gases are swept clear from the mold before the mold is completely filled. In the teeming operation the workmen pouring the steel watch the flames shooting from the openings 12 and 14 beneath the fountain and when these flames cease it is an indication that the mold is filled and no more 95 gas is escaping, at which time the teeming operation is stopped.

Since the side walls of the mold are proportioned to provide a large heat absorbing capacity which is substantially uniform around the mold matrix, an enclosing shell of chill steel quickly forms from the molten mass and builds up in thickness so that if 100 the occluded gases in the steel are not completely driven from the steel before the mold is filled these gases are enclosed by the shell and are driven inward under pressure from the enclosing solidifying steel walls. It 105 sometimes happens that a zone of gas bubbles will thus be formed an inch and a half or more from the outer wall of the ingot. As the ingot continues to cool pressure conditions are changing in the ingot and it appears that no further gas bubbles tend to 110 form so that the center of the ingot is substantially solid metal.

When the clamps are loosened and the mold opens, the runner tile leaves the mold 115 with the ingot, since the runner tile sets tightly against the ingot the runner tile inlets are short and the scrap therefore is relatively small.

Figure 6 is a longitudinal section through 120

an ingot on which are indicated zones A, which represent zones of isocrystallization. It will be noted that these zones are closed shell like areas which are substantially coincident with the general shape of the ingot and are substantially uniform for both ends of the ingot as well as substantially symmetrical to the axes thereof. The zone B indicates a zone of gas bubbles and shows the general direction of such bubbles as being at right angles to the surface of the ingot adjacent thereto.

Figure 7 is a cross-section through an ingot in accordance with the present invention likewise indicating the zones of isocrystallization A and the gas bubbles B and with the corner C thereof being that portion of the ingot which occupies the uppermost part of the mold matrix. From these views it will appear that the isocrystallization zones are substantially symmetrical to the axes of the ingot and with the zones comprising closed areas. In this ingot the outer shell is substantially pure steel and the materials which otherwise would segregate are forced inward during the cooling action, and since pressure conditions on the interior of the ingot change during cooling, segregation seems to be prevented and substantially uniform metal occurs in the middle of the ingot.

The present invention provides a steel ingot wherein all sides thereof are smooth and comprise rolling surfaces, and the gas bubbles such as form are so deep seated in the ingot that rolling welds the cavities together and therefore the present ingot is adapted to be rolled into a substantially one hundred per cent product thereby obviating loss due to cropping of the ingot.

Having thus described my invention, what I claim is:

1. As an article of manufacture an ingot of steel or the like having a substantially uniform deep chilled shell on all longitudinal sides and at both ends and with the chill being substantially symmetric throughout the length of the ingot.

2. As an article of manufacture an ingot of steel or the like having a substantially uniform deep chilled shell on all longitudinal sides and at both ends and with the chill being substantially symmetric throughout the length of the ingot, with the sides and ends of the ingot smooth and substantially all gas bubbles being deep seated therein so that said ingot may be rolled into finished product without cropping the ingot.

3. As an article of manufacture an ingot of steel or the like having a substantially uniform chilled shell on all sides and at both ends and with the chill being substantially symmetric throughout the length of the ingot, with the sides and ends of the ingot smooth and substantially all gas bubbles being deep seated therein between the outer

shell and a solid metal core containing a higher percentage of metalloids than the chilled shell.

4. As an article of manufacture a steel ingot having smooth sides and ends with all sides and ends uniformly deep chilled.

5. As an article of manufacture a steel ingot having smooth sides with all longitudinal sides uniformly deep chilled and having a solid metal core containing a higher percentage of metalloids than the deep chilled sides.

6. The method of casting steel ingots having a plurality of longitudinally extending sides which comprises casting the ingot with the major axis thereof substantially horizontal and with the apex of the angle formed by two sides thereof comprising the highest portion of the mold into which gases may collect, draining the gases from the mold adjacent a portion of said apex, and chilling the opposite ends of the ingot at substantially the same rate.

7. The method of casting steel ingots having a plurality of longitudinally extending sides which comprises casting the ingot with the major axis thereof substantially horizontal and with the apex of the angle formed by two sides thereof comprising the highest portion of the mold into which gases may collect, draining the gases from the mold adjacent a portion of said apex, and chilling the sides and ends of the ingot at substantially the same rate.

8. The method of casting steel ingots or the like which comprises casting the ingot with the major axis substantially horizontal and with a diagonal axis substantially vertical introducing steel adjacent the highest portion of one end of the mold and causing expelled gases to escape from the mold at the same end thereof at which the molten steel is introduced.

9. The method of casting steel ingots or the like which comprises casting the ingot with the major axis inclined slightly to the horizontal and with a diagonal axis substantially vertical, introducing molten steel adjacent the highest portion of one end of the mold, and causing expelled gases to escape from the mold at the same end thereof at which the molten steel is introduced.

10. The method of casting steel ingots having a plurality of longitudinally extending sides which comprises casting the ingot with the major axis thereof substantially horizontal and with the apex of the angle formed by two sides thereof comprising the highest portion of the mold into which expelled gases may collect, and draining the expelled gases from the mold adjacent a portion of said apex.

11. The method of casting steel ingots having a plurality of longitudinally extending sides which comprises casting the ingot

- with the major axis thereof inclined slightly to the horizontal and with the apex of the angle formed by two sides thereof comprising the highest portion of the mold into 5 which expelled gases may collect, and draining the expelled gases from the mold adjacent a portion of said apex.
12. The method of casting steel ingots having a plurality of longitudinally extending sides which comprises casting the ingot with the major axis thereof substantially horizontal and with the apex of the angle formed by two sides thereof comprising the highest portion of the mold into which expelled gases may collect, pouring the steel in such manner as to cause the steel to rise vertically and to sweep gas bubbles from beneath the angularly disposed sides, and draining the expelled gases from the mold 10 adjacent a portion of said apex.
13. The method of casting steel ingots and the like comprising casting the ingot with the major axis thereof substantially horizontal and with the lowermost portion 15 of the ingot comprising the apex of an angle forming an edge by the meeting of two sides of the ingot and with the uppermost portion of the ingot comprising the apex of an angle also formed by the meeting of two sides of 20 an ingot.
14. The method of casting steel ingots and the like comprising casting the ingot with the major axis thereof substantially horizontal and with the lowermost portion 25 of the ingot comprising the apex of an angle forming an edge by the meeting of two sides of the ingot and with the uppermost portion of the ingot comprising the apex of an angle also formed by the meeting of two sides of an 30 ingot, and uniformly chilling the steel upon all sides of the ingot to cause gas bubbles to be deep seated therein.
15. The method of casting steel ingots which comprises casting the ingot with the major axis thereof substantially horizontal and with a diagonal axis thereof substantially vertical, and permitting gases to escape from the mold during casting through 35 an opening arranged to lie substantially on said diagonal axis.
16. The method of casting steel ingots which comprises setting a closed horizontal mold with a diagonal of the matrix portion vertical and the longitudinal axis inclined 40 slightly to the horizontal, then filling the matrix with molten steel.
17. The method of casting horizontal steel ingots which comprises flowing the molten steel from a plurality of openings in different vertical portions of a single runner, 45 into a chill mold matrix having the longitudinal axis inclined to the horizontal.
18. The method of casting horizontal steel ingots which comprises flowing the molten steel from a plurality of openings in dif- 50 ferent vertical portions of a single runner, 55 into a chill mold matrix having the longitudinal axis inclined to the horizontal and permitting the mold gases to escape around the runner. 70
19. The method of casting horizontal steel ingots which comprises flowing the molten steel into a mold matrix from a plurality of openings arranged at different vertical heights, and providing a gas outlet extending across one end of the matrix in such manner that said outlet is sealed as the steel rises. 75
20. The method of casting horizontal steel ingots which comprises flowing the molten steel into a mold matrix from a runner having a plurality of openings arranged at different vertical heights, and providing a gas outlet around the runner and extending across one end of the matrix in such manner that said outlet is sealed as the steel rises. 80
21. An ingot mold for casting horizontal ingots comprising a plurality of sections with the separation plane of said sections arranged on a diagonal of the matrix portion of the mold and with the highest part of the matrix portion of the mold comprising the apex of an angle formed by two sides of the matrix. 85
22. An ingot mold for casting horizontal ingots comprising a plurality of sections with the separation plane of said sections arranged on a diagonal of the matrix portion of the mold and with the highest part of the matrix portion of the mold comprising the apex of an angle formed by two sides of the matrix and having the longitudinal axis of the matrix inclined slightly to the horizontal. 90
23. An ingot mold for casting horizontal ingots comprising a plurality of sections with the separation plane of said sections arranged on a diagonal of the matrix portion of the mold and with the highest part of the matrix portion of the mold comprising the apex of an angle formed by two sides of the matrix and having the longitudinal axis of the matrix inclined slightly to the horizontal and with the outside surfaces of the mold being substantially inclined at forty-five degrees to the plane of adjacent side surfaces of the matrix to provide walls having large heat absorption capacity adjacent the side of the matrix. 95
24. A mold for casting steel ingots having walls to chill the ingot and with a section of the mold wall adjacent a matrix surface being substantially triangular to provide a uniform chill around the matrix and to cause the sides of an ingot to chill at substantially the same rate as the corners. 100
25. A mold having a body portion with a matrix to cast an ingot, said body portion being formed with an opening to re- 105
- 110
- 115
- 120
- 125
- 130

ceive a runner, and a runner extending into said opening with a plurality of discharge outlets in said runner and located at different vertical heights.

5 26. A chill mold for casting horizontal ingots that are polyhedral in cross-section, with the heat absorbing capacity of the walls of the mold being high and so proportioned that the sides of the matrix of the 10 mold will absorb heat at substantially the same rate as the corners thereof.

27. A chill mold for casting steel ingots with the matrix arranged therein with one diagonal of the matrix being substantially 15 vertical and another diagonal being substantially horizontal and with the walls of the mold arranged to have a heat absorbing capacity which is greater at the ends of the said vertical diagonal than at the ends of 20 the horizontal diagonal.

28. A chill mold for horizontal ingots having a matrix therein and with the heat absorbing capacity of the mold walls being slightly greater in the upper half of the 25 mold than in the lateral portions thereof to provide a deep chill on the top of the ingot and cause gas bubbles to be deep seated therein.

29. The method of casting steel ingots 30 which comprises causing the steel to form in a pool the surface of which first increases in width and then decreases in width, symmetrical portions being formed during the decreasing and increasing stages, then 35 quickly chilling the metal in the pool in such manner as to drive a portion of the metalloids toward the central part of the steel mass and to enclose occluded gases within the steel mass.

30. The method of casting steel ingots 40 which comprises providing a substantially horizontal mold having a substantially square cross-section matrix, arranging said matrix with one diagonal thereof substantially vertical, quickly filling said matrix 45 with molten steel and maintaining the steel mixed during the filling operation, then quickly chilling the exterior of the steel mass to form a shell enclosing the molten interior and causing the shell to cool with sufficient 50 rapidity to establish internal pressure on the molten mass to prevent formation of gas bubbles near the surface of the ingot.

31. The method of casting steel ingots

which comprises casting the ingot in a substantially horizontal mold through a removable runner at one end of the mold matrix which runner is adapted to leave the mold with the ingot when the mold is opened after the ingot is frozen.

32. As an article of manufacture comprising an ingot chill mold adapted to enclose all sides of the ingot and having a substantially rectangular cross-sectional to the matrix, the chill metal in the sides of said mold being uniformly proportioned so as to absorb heat at substantially the same rate as the corner portions of the mold between said sides.

33. As an article of manufacture an ingot of steel having rollings surface throughout the length thereof comprising an inner core of a higher percentage of metalloids than the outer surrounding portion or shell and with the gas bubbles in the ingot confined to a zone lying between said core and shell.

34. An article of manufacture an ingot of steel comprising a core containing a higher percent of metalloids than the outer shell of the ingot and with a zone of gas bubbles confined to a portion between the core and shell, with the gas bubbles disposed substantially uniformly relatively to the longitudinal axis of the ingot.

35. As an article of manufacture a steel ingot comprising a mass of steel with the surface thereof shaped by a mold and with the sides substantially parallel and comprising rolling surfaces throughout the length of the ingot, and with the center of said ingot comprising a substantially solid core of a higher percentage of metalloids than outer surfaces or shell of said ingot.

36. An ingot mold for casting horizontal ingots comprising a plurality of sections with the longitudinal lines of separation of said sections arranged one above the other on a diagonal of the matrix portion of the mold and with the highest part of the matrix portion of the mold comprising the apex of an angle formed by two sides of the matrix.

37. A chill mold for casting horizontal ingots comprising a substantially prism-shaped matrix bounded by chilling end walls and chilling side walls, and with a corner of said matrix forming the highest part thereof.

JOHN E. PERRY.